

# UNITED STATES PATENT OFFICE.

VIGGO ANTON FRYDENBERG, OF TISVILDELEJE, DENMARK.

## METHOD OF TREATING SEA-TANG.

1,322,237.

Specification of Letters Patent.

Patented Nov. 18, 1919.

No Drawing.

Application filed April 9, 1918. Serial No. 227,537.

*To all whom it may concern:*

Be it known that I, VIGGO ANTON FRYDENBERG, citizen of the Kingdom of Denmark, residing at Tisvildeleje, in the county of 5 Sjælland and State of Denmark, have invented certain new and useful Improvements in Methods of Treating Sea-Tang, of which the following is a specification.

The invention consists in a method of 10 treating sea-tang, especially grass-wrack (*Zostera marina*) to make the same fit for use as pulp in the paper manufacture instead of or together with the so called mechanical or chemical cellulose and for dif- 15 ferent other uses, for instance as addition to plaster, stucco and the like to strengthen the same.

To this end the fresh, moist sea-tang is exposed to the influence of chlorin or any other 20 suitable bleaching agent, such as for example slaked lime or the like, which has the effect that the sea-tang becomes white or whitish-gray. Afterward it is dried in the air or artificially and finally—according to 25 the use which is to be made of the material—rent asunder or crushed to a suitable degree of fineness.

According to the invention the treatment 30 with chlorin, chlorid of lime and the like takes place, not as by the until now known methods of this sort so thoroughly that a separation of certain ingredients of the tang takes place; but the treatment is limited to the bleaching only, without any other spe- 35 cial chemical influence on the tang being aimed at. It is hereby effected that the whole mass of tang can be applied in the paper manufacture and an application of the parts of the tang, which by the formerly

known methods for the treatment of tang 40 were separated as a residual product of little use, becomes possible.

Instead of treating the sea-tang in fresh state one may also treat the tang after it has been dried and then moistened. 45

If chlorin is to be applied for the bleaching this may suitably take place by arranging the sea-tang in thin layers, covered with chlorid of lime whereafter the tang is allowed to lie a short time under influence of 50 this chemical.

By the application of sea-tang in the manufacture of for instance colored paper, stucco, pasteboard-pulp and the like, by which it is of no importance to obtain a 55 white or very light product the sea-tang may with advantage be applied without any foregoing bleaching, as hereby a considerably stronger product is obtained.

Having now particularly described and 60 ascertained the nature of my said invention I declare that what I claim is:

A method of treating sea tang to prepare it for paper manufacture and other uses consisting in first subjecting fresh or moistened 65 sea tang to the action of a bleaching agent to a degree insufficient to disorganize it or separate its elements and afterward drying and comminuting the bleached sea tang so that all parts of it may be available in the 70 pulp.

In testimony whereof, I have signed my name to this specification in the presence of two subscribing witnesses.

VIGGO ANTON FRYDENBERG.

Witnesses:

MAGNUS JENSEN,  
ERVIN JACOBSEN.